

W. H. HOWARD.

PROCESS FOR OBTAINING A CONTINUOUS FLOW OF SO<sub>2</sub> FROM WHITE METAL.

APPLICATION FILED MAR. 10, 1920.

1,377,013.

Patented May 3, 1921.



*WITNESSES:*

W. H. H. H.

INVENTOR  
William A. Howard  
BY  
Albert M. Austin  
ATTORNEYS

# UNITED STATES PATENT OFFICE.

WILLIAM H. HOWARD, OF SALT LAKE CITY, UTAH, ASSIGNOR TO AMERICAN SMELTING AND REFINING COMPANY, OF NEW YORK, N. Y., A CORPORATION OF NEW JERSEY.

## PROCESS FOR OBTAINING A CONTINUOUS FLOW OF SO<sub>2</sub> FROM WHITE METAL.

1,377,013.

Specification of Letters Patent.

Patented May 3, 1921.

Application filed March 10, 1920. Serial No. 364,836.

To all whom it may concern:

Be it known that I, WILLIAM H. HOWARD, a citizen of the United States, and resident of Salt Lake City, in the county of Salt Lake and State of Utah, have invented certain new and useful Improvements in Processes for Obtaining a Continuous Flow of SO<sub>2</sub> from White Metal, of which the following is a specification.

10 The invention relates in general to a process of obtaining a practically continuous stream of gas of high sulfur dioxid contents from the gases formed in blowing copper matte in a converter, with the object of recovering the sulfur dioxid.

The invention also relates to an improved form of instrumentality for economically and efficiently practising the method feature of the present disclosure.

20 It has been suggested in my prior application on process for recovering sulfur dioxid, Serial No. 233,640, filed May 10, 1918, that copper matte be treated in one set of converters until reaches what is known as 25 "white metal," and at which stage the converter gas is of a character to permit the profitable recovery of the sulfur dioxid therefrom and then this "white metal" be removed to a separate converter or preferably a plurality of converters in which the recovery process is carried on. The present disclosure constitutes an improvement over the method suggested in the above identified application wherein the necessity for removing the white metal from one converter 30 into another has been avoided and the method is carried on continuously in one converter or rather in a battery of such converters so as to insure the continuity of 35 a uniform supply.

One of the objects of the invention therefore is to provide a continuous supply of high grade sulfur dioxid gas, with the elimination of the carrying from one place 45 to another of hot material and the avoidance of resulting temperature losses.

Broadly, I attain these objects by separating the sulfur containing material, such as the copper matte mentioned into batches 50 and successively treating each batch to a preliminary blowing operation as is usual in copper converting to blow off the gases which are low in sulfur dioxid content, and then to continue the blow to drive off and

retain the gases which are relatively high in 55 sulfur dioxid content. The operation on each succeeding batch is carried on in such a timed sequence that each succeeding batch will be producing gas at the desired richness of sulfur dioxid content by the time 60 the gas from the preceding batch is beginning to fall below the desired content of sulfur dioxid gas.

In one commercially perfected plant the 65 low grade gases are caused to discharge into a conduit from which they may be conveyed to a Cottrell plant or bag house, or other devices for suitable treatment usual with 70 gases of this character and the discharge from the several batches of material under 75 treatment is intercepted when the batches reach that point where it is desirable to retain the high grade sulfur dioxid content. The high grade sulfur dioxid gases are then directed into some common receptacle or 80 conduit and suitable control is provided so that the supply from any one batch may be cut off from the common receptacle when the content of any one batch falls below the requisite amounts desired in the conduit. 85

Referring to the apparatus features of the disclosure, the primary object of the invention when considering this aspect thereof is to provide a simple form of plant for controlling the different stages of the 85 gas discharge and for providing a simple means for practising the method economically and with the minimum loss of heat or of gases.

Referring to the accompanying drawings 90 for a diagrammatic showing of a plant for practising the method disclosed and for illustrating a preferred embodiment of the physical features of the invention, the drawing is a diagrammatic view in side elevation of a flow line in a commercial plant.

In the drawings there is shown a battery 100 of converters 10, herein shown to be four in number which number has been found to be admirably adapted to carry out the process 100 in one plant. Each of the converters is connected by means of a hood or end connection 11, such as is shown in my copending application, Serial No. 342,451, filed December 4, 1919, with a main gas conduit 105 12 common to all of the converters and leading to a bag house 13 or other receptacle or device for receiving the high grade gases

and dust discharged from the converters. Each of the conduits 11 is controlled by valve 14, so that any one of the converters may be opened at will to the conduit 12, 5 which leads to the sulfur dioxid recovery plant.

Each of the converters is also provided with another gas conveying pipe 15, leading to a conduit 17, for conveying the gases to 10 a dust and fume recovery plant, then wasting to the atmosphere, or directly wasted to the atmosphere without a special dust or fume recovery plant.

In one commercial operation of the method 15 disclosed it is usual to continue the preliminary blowing, discharging the waste gases into the conduit 17 until the mass in the converter has reached the stage known as "white metal," at which time the second 20 converter is started and the first converter is opened to the high  $\text{SO}_2$  gas supply conduit 12. When the gas from the first converter begins to fail, the charge in the second converter has nearly reached, or has 25 reached the white metal stage; then the gas from this converter is delivered to the high  $\text{SO}_2$  main, and the first converter is charged with fresh matte, and the operation alternately repeated, so that a practically continuous 30 supply of high grade gas is delivered to the  $\text{SO}_2$  recovery plant.

Having thus described my invention, I claim:

1. In the art of recovering sulfur dioxid 35 from white metal, the process which consists in subjecting a plurality of bodies of copper matte successively to a blowing operation to drive off gases having a relatively low sulfur dioxid content and then continuing 40 the blow through each body to recover gases having a relatively high sulfur dioxid content, maintaining the sequence of operation in a timed relation to provide a continuous flow of gases having high sulfur dioxid content from the plurality of bodies of copper 45 matte.

2. In the art of providing a continuous supply of gas having a relatively high sulfur dioxid content, the process which consists in treating a batch of copper matte to 50 drive off gases having a relatively low sulfur dioxid content, similarly treating another body of copper matte in such timed relation to the treatment in the first named body that 55 the removal of low grade sulfur dioxid gas in the second body will be subsequent to the removal in the first named body, blowing said first named body to provide a flow of gas having a relatively high sulfur dioxid 60 content and similarly blowing the second named body in time to maintain a continuation of the flow of high grade sulfur dioxid gas as the flow from the first named body becomes exhausted.

3. In the art of providing for a continuous

supply of gas having a relatively high sulfur dioxid content, the process which consists in treating a batch of a sulfur containing substance for a period of time to remove the gases having a relatively low sulfur 70 dioxid content, continuing the treatment to obtain a flow of gas having a relatively high sulfur dioxid content for the period of time that the gas recovered maintains its high grade, collecting said high grade gas, similarly treating another batch of said substance in such timed relation that the high grade gases from the second batch will be available to continue the flow into the collecting means as the gases from the first 80 named batch begin to fail in maintaining the supply of high grade gas.

4. In the art of providing for a continuous supply of gas having a relatively high sulfur dioxid content, the process which consists in subjecting a plurality of sulfur containing substances first to a preliminary treatment to remove gases having a relatively low sulfur dioxid content and then successively subjecting the substances to a 90 treatment to remove gases having a relatively high sulfur dioxid content and collecting said gases from succeeding batches as the gas supply from a preceding batch begins to fail.

5. In the art of recovering a high grade sulfur dioxid containing gas from copper matte, the process which consists in treating a bath of the matte to the actions of an air blast to drive off gases having a relatively 100 high sulfur dioxid content, similarly treating a second batch of matte in time to maintain a continuity of supply when the supply from the first batch falls below a definite sulfur dioxid content and similarly treating 105 a third batch to maintain the flow from the second batch while permitting the flow from the first batch to be intercepted.

6. The process of recovering sulfur dioxid from copper matte, which consists in successively treating different batches of the matte each for a predetermined time to remove the sulfur dioxid therefrom and without interruption between the periods of time, and continually collecting said sulfur dioxid to 115 maintain a substantially constant supply of gas.

7. The process of recovering sulfur dioxid which consists in successively subjecting different batches of sulfur containing substances to a preliminary treatment to remove gases having a relatively low sulfur dioxid content, then successively treating the different batches to remove gases having a relatively high sulfur dioxid content, and continuously collecting the high grade gases from the different batches as they successively begin to discharge the high grade gas thereby to maintain a substantially constant 120 supply of gas.

8. The process of recovering sulfur dioxid containing substances, the process which consists in successively subjecting different batches of the substances to a preliminary treatment to remove gases having relatively low sulfur dioxid content, then successively treating the different batches to remove gases having a relatively high sulfur dioxid content said preliminary treatment and the 5 succeeding gas eliminating treatment being continuous with each batch and continuously collecting the high grade gases from the different batches as they successively begin to discharge the high grade gas thereby to 10 maintain a substantially constant supply of gas.
9. The process of recovering a constant substantially uniform supply of sulfur dioxid gas which consists in treating a sufficient quantity of white metal to give off a 15 predetermined quantity of gas having a relatively high and substantially uniform sul-

fur dioxid content, similarly treating another such quantity in a timed relation to maintain a continuity of the supply of gas 25 from the first named treatment and of approximately the same composition.

10. In the art of recovering a constant and substantially uniform supply of sulfur dioxid from copper matte the process which 30 consists in successively blowing different portions of the matte until the gases produced from each portion have a predetermined composition, continuing the blow for a period of time to recover the gas having 35 said desired composition, said periods of time being continuous and one following the other in order, whereby a continuous flow of gas is obtained having a substantially uniform composition. 40

Signed at Salt Lake City, in the county of Salt Lake, and State of Utah this 19th day of February, A. D. 1920.

WILLIAM H. HOWARD.